

June 6, 1961

V. R. PALMERI  
PRESSURE RESPONSIVE RESISTOR

2,987,687

Filed April 28, 1960

FIG. 1



FIG. 2



INVENTOR.  
VICTOR R. PALMERI  
BY  
*Philip G. Gilbert*  
ATTORNEY

# United States Patent Office

2,987,687

Patented June 6, 1961

1

2,987,687

## PRESSURE RESPONSIVE RESISTOR

Victor R. Palmeri, Weehawken, N.J., assignor to Space Dynamics Corporation, Clifton, N.J., a corporation of New Jersey

Filed Apr. 28, 1960, Ser. No. 25,462

12 Claims. (Cl. 338—36)

This invention relates to pressure responsive resistors, and more particularly, concerns devices sensitive to changes of applied pressure and adapted to vary its electrical resistance in accordance with such changes in pressure.

In electrical or electronic circuitry it is frequently desirable to include as a component thereof resistor means whose resistance values change in accordance with pressures applicable to the component. Thus with instrumentation controls regulation thereof may be responsive to pressure conditions as well as other environmental factors or characteristics.

Accordingly, an object of this invention is to provide an improved pressure responsive resistor which is compact and of minimum bulk, which may be readily accommodated to small or irregular spaces, and which shows high sensitivity to small changes in pressure.

Another object of this invention is to provide in a device of the character described, a body of material of predetermined composition which is operative to sense small variations in pressure applied to the body and to change its resistance accordingly.

A further object of this invention is to provide in a device of the character described, a pressure responsive element in the form of a layer of material whose composition may be adjusted in accordance with the magnitudes of the pressure ranges to be sensed.

Still another object of this invention is to provide a pressure responsive resistor in flat, flexible form which is readily adapted to conform to supporting surfaces of varying shape, yet is highly sensitive to variations in pressure so as to change its resistance values.

Other objects of this invention will in part be obvious and in part hereinafter pointed out.

In the drawing, FIG. 1 is an enlarged transverse sectional view of a device embodying the invention;

FIG. 2 is a top plan view thereof.

Essentially, the device of the instant invention comprises a body of material of predetermined composition; the body being suitably enclosed and provided with electrodes or terminals in contact with opposite surface portions of the body. The assembly may be in thin flat form and may be flexible so as to readily conform to an irregular supporting surface. The body of material is made up as a particulate mixture of silicon and rare earth compounds, such as the oxides; the oxide being present in relatively small amounts.

The body of material may have its composition adjusted by the addition of small amounts of powdered metal and inert fillers, to suit particular pressure ranges; and may also contain small amounts of a flexible binder.

Thus, as shown in FIGS. 1, 2; a pressure responsive resistor embodying the invention, is generally shown at 10. The same is in flat strip form comprising a pair of opposed strips 11, 12 of synthetic resin such as Teflon (polytetrafluoroethylene), polystyrene, vinyl, copolymer or the like. The strips 11, 12 enclose and seal a body 13 of predetermined composition; electrodes or terminals 14, 15 being disposed in contact with body 13 on opposite sides thereof.

The body 13 is made up in the form of a mixture of silicon and a small amount of a rare earth compound such as the oxide of gadolinium, neodymium, samarium, scandium or yttrium. The silicon may be present in amounts

2

ranging from about 90 to about 99%; the rare earth oxide in amounts of from about 0.1 to about 10%. Filler such as silicon dioxide or zirconium dioxide may also be added in amounts of from about 1 to about 10%. Also, in some instances, the mixture may include small amounts of powdered tungsten, nickel or chromium, ranging up to about 3%.

Thus, in a resistor 10 for sensing variations of pressure within a relatively high pressure range, body 13 may be made up of 92% silicon, 4% gadolinium oxide and 4% zirconium dioxide. The several materials are thoroughly admixed in particulate form and then suitably agglomerated in thin sheet or block form for assembly with strips 11, 12.

15 Strips 11, 12 are previously treated on one surface thereof to form electrodes 14, 15 thereon, as by cathode sputtering of electrodeposition of a suitable metal film to constitute said electrodes; which may be of silver, gold, platinum or the like. Wire leads 16, 17 may extend from electrodes 14, 15, to provide electrical connecting means.

The strips 11, 12 with body 13 therebetween, are sealed together by a suitable elastic sealant 18 extending about the periphery of said strips and adhering their opposed marginal edge portions. Sealant 18 may be of a rubbery 25 or plastic character and preferably of a chemical resistant nature.

Another formulation for body 13 comprises 96% silicon, 1% yttrium oxide and 3% silicon dioxide. The formulation was prepared in agglomerated form and assembled with enclosing strips 11, 12, as previously described. Such device is particularly effective for intermediate pressure ranges.

For relatively low pressure ranges, body 13 may be made up of 98% silicon, 0.5% gadolinium oxide, 0.3% zirconium dioxide, 0.2% rubber binder and 1% tungsten powder.

The material making up body 13 is in powdered form with a particle size ranging from about .0001 to about .025". Upon adding small amounts of plastic elastic 40 binder, the resultant flexible body together with its flexible enclosure may be readily mounted on curved or irregular surfaces.

As various changes might be made in the embodiments of the invention herein disclosed without departing from the spirit thereof, it is understood that all matter herein shown or described shall be deemed illustrative and not limiting except as set forth in the appended claims.

Having thus disclosed my invention, I claim as new and desire to protect by Letters Patent:

50 1. A pressure responsive resistor comprising a flexible body of material and a pair of electrodes respectively in contact with opposite portions of said body, said body comprising a major portion of silicon and a minor portion of a rare earth material selected from the group consisting of gadolinium, neodymium, samarium, scandium and yttrium oxides.

55 2. A pressure responsive resistor comprising a body of material and a pair of electrodes respectively in contact with opposite portions of said body, said body comprising a major portion of silicon and a minor portion of a compound selected from the group consisting of gadolinium, neodymium, samarium, scandium and yttrium oxides.

60 3. A resistor as in claim 2 wherein said body further includes a minor amount of powdered metal.

4. A resistor as in claim 2 wherein said body further includes a minor amount of elastic binder.

65 5. A resistor as in claim 2 wherein the silicon is present in amounts of from about 90 to about 99% and the oxide is present in amounts of from about 1 to about 10%, all by weight.

70 6. A resistor as in claim 2 wherein said body comprises

agglomerated particles, said particles having a size of from about .0001 to about .025".

7. A pressure responsive resistor comprising a body of material, a sealed enclosure for said body of material, said enclosure comprising electrical insulating sheet material, metal film electrode means on the inner surface portions of said enclosure and in contact with opposed surface portions of said body of material, said body of material comprising a major portion of silicon and a minor portion of a rare earth material selected from the group consisting of gadolinium, neodymium, samarium, scandium and yttrium oxides.

8. A resistor as in claim 7 wherein said body of material further includes a minor portion of elastic binder.

9. A resistor as in claim 7 wherein said enclosure comprises synthetic resin sheeting.

10. A resistor as in claim 8 wherein said sheeting is formed of polytetrafluoroethylene.

11. A resistor as in claim 7 wherein said rare earth oxide is gadolinium oxide.

12. A resistor as in claim 7 wherein said silicon is present in amounts of from about 90 to about 99% by weight.

10

References Cited in the file of this patent

## UNITED STATES PATENTS

1,039,463 Thomson Sept. 24, 1912